

## 1

3,009,843

STEEL PRODUCTS AND METHOD FOR  
PRODUCING SAME

Elliot S. Nachtman, Park Forest, Ill., and John E. O'Donnell, Highland, Ind., assignors to LaSalle Steel Company, Hammond, Ind., a corporation of Delaware  
No Drawing. Filed Oct. 22, 1956, Ser. No. 617,267

13 Claims. (Cl. 148—12.1)

This invention relates to the improvement of mechanical and physical properties of steel in a process which is capable of use in the cold-finishing of steel, as in the cold-finishing of steel bars, rods, wires, tubing, and the like steel products.

It is an object of this invention to produce and to provide a method for producing cold-finished steel products having new and improved physical properties, and it is a related object to produce a new and improved steel product having combinations of characteristics which differ from steels which have heretofore been produced.

More specifically, it is an object of this invention to provide a method applicable to the metallurgical processing of a hot-rolled steel, such as a steel of the type which strain-hardens and hardens by some mode of precipitation when worked at elevated temperatures to improve the physical and mechanical properties of the steel.

This application is an improvement over the copending applications Serial Nos. 518,411, 518,412, now Patent Nos. 2,767,837 and 2,767,835, respectively, both granted October 23, 1956, 518,413, and 518,414, now Patent Nos. 2,767,836 and 2,767,838, respectively, both granted October 23, 1956, filed by Nachtman and Moore on June 27, 1955.

In the aforementioned copending applications, the teaching is made of the new and improved concept for enhancing the physical and mechanical properties of steel by the combination of steps which includes the step of advancing the steel through a die to effect reduction in cross-sectional area while the steel is at a temperature within the range of 200° F. to the lower critical temperature for the steel composition. This step is referred to hereinafter as the elevated-temperature-reduction step, which is effected by working the steel to effect reduction in cross section while the steel is at a temperature within the range of 200° F. to 1100°—1200° F. In accordance with the teaching of the aforementioned copending applications, the temperature employed in the elevated-temperature-reduction step influences the trend of improvements secured in physical and mechanical properties of the steel. By controlling temperature, chemistry, and the amount of reduction, it becomes possible selectively to vary physical and mechanical properties developed in the steel. The properties can be varied over a fairly wide range while enhancing and improving the uniformity of physical and mechanical characteristics developed in steels of the same chemistry from heat to heat, as distinguished from the wide variations which normally exist in hot-rolled steels.

It has now been found that the high-strength levels secured by elevated-temperature reduction of steels, as defined in the aforementioned copending applications, can be maintained along with many of the other improvements made available in the steels by the elevated-temperature-reduction step, and that still further improvements can be secured in the physical and mechanical properties of the steel to produce new and improved steel products when use is made of a combination of steps which includes heat-treating the steel after the elevated-temperature-reduction step.

As used herein, the term "heat treatment" after elevated-temperature reduction is meant to include:

(1) Annealing the steel after the elevated-temperature-reduction step by heating the steel to annealing temperature or to a temperature in the range of 1400°—1500° F.

## 2

followed by slow cooling, as by means of air, to room temperature similarly to the annealing step employed in advance of elevated-temperature reduction.

(2) Normalizing the steel after the elevated-temperature-reduction step by heating the steel to normalizing temperature or to a temperature (above the upper critical temperature of the steel) between 1300° and 1500° F. followed by rapidly cooling the steel to room temperature.

(3) Producing a phase change in the steel after the elevated-temperature-reduction step by heating the steel to a temperature above the transformation range—that is, to a temperature in the order of 1500°—1600° F. and then quenching the steel to room temperature to produce a phase change to martensite.

(4) Producing a phase change in the steel after taking the elevated-temperature-reduction step, as by heating the steel to a temperature above the transformation range such as to a temperature within the range of 1500° to 1600° F., quenching the austenitized steel and then tempering the quenched steel by re-heating the steel to form tempered martensite.

(5) Processing the steel after the elevated-temperature reduction step by heating the steel to a temperature above the transformation range, such as to a temperature within the range of 1500°—1600° F., followed by a partial quench to a temperature within the range of 200° F. to the lower critical temperature for the steel composition.

(6) Mar tempering the steel after taking the elevated temperature reduction, as by heating the steel to a temperature above the transformation range, that is, to a temperature above 1500° F. and then quenching the steel in a bath maintained at a temperature in the upper portion of the temperature range for martensite formation ( $M_s$ ) until the metal has reached that temperature and then the steel is allowed to cool through the range for martensite formation to ambient temperature.

(7) Austempering the steel after taking the elevated temperature-reduction step by heating the steel to a temperature above the transformation range, such as to a temperature within the range of 1500°—1600° F. followed by quenching the steel in a bath maintained at a temperature slightly above the  $M_s$  range and of a character which causes the extraction of heat from the steel at a rate which prevents passage of the steel through the austenitic range or prevent high temperature transformation products, and maintaining the steel at a temperature below that of pearlite formation but above that of martensite formation, such, for example, as when the steel is quenched in a salt bath maintained at a temperature of 640° F. followed by quenching to room temperature after the temperature of the steel has become uniform at the temperature of the quench.

(8) Treating the steel by diffusion transfer, as, for example, in the processes of carburizing, nitriding, cyaniding, chromizing, and carbonitriding the steel after the steel has been processed to the elevated-temperature-reduction step. As used herein, the terms "diffusion" and "carburizing" are intended to have their normal meaning in the steel trade. Diffusion can be defined briefly as involving the movement of atoms within a solution. The net movement is usually in the direction from regions of high concentration towards regions of lower concentration in the attempt to achieve homogeneity of the system, which may be in a liquid or gas or, as in the present instance, a solid metal. Carburizing is a diffusion transfer process wherein carbon is introduced into the steel by bringing the steel into intimate contact in relation with a carbonaceous material, in the form of solid, liquid or gas, and heating to a temperature above the transformation range for the steel and holding



The steel, at the desired elevated temperature, was then lubricated with a conventional drawing compound and advanced through the draw die to take a representative reduction in cross-sectional area. The 1144 steel, originally of  $\frac{5}{8}$ " round, was given a 21.6% reduction, while the 4140 steel, of  $1\frac{1}{16}$ " round, was given a 19.9% reduction.

After the elevated-temperature-reduction step, the steels were heated to austenitizing temperature for one hour. The temperature employed was  $1500^{\circ}$  F., and then the austenitized steels were quenched in oil to room temperature.

Table I

C-1144—

Drawn to take a 21.6% reduction  
Austenitized at  $1,500^{\circ}$  F. for one hour  
Quenched to room temperature

| Temp. of draw,<br>° F. | Austen-<br>itizing<br>temp.,<br>° F. | Tensile<br>strength,<br>p.s.i. | Izod<br>impact<br>70° F.<br>ft.-lbs. | Hardness |     |     | Warp-<br>age |
|------------------------|--------------------------------------|--------------------------------|--------------------------------------|----------|-----|-----|--------------|
|                        |                                      |                                |                                      | S        | MR  | C   |              |
| Hot roll.....          | 1,500                                | 224,000                        | 11.7                                 | 597      | 475 | 473 | $\pm .127$   |
| Cold drawn.....        | 1,500                                | 294,000                        | 12.0                                 | 610      | 642 | 610 | $\pm .208$   |
| 500.....               | 1,500                                | 254,000                        | 10.7                                 | 626      | 531 | 531 | $\pm .223$   |
| 1,000.....             | 1,500                                | 248,500                        | 4.7                                  | 619      | 513 | 502 | $\pm .181$   |

Table II

C-4140—

Drawn to take a 19.9% reduction  
Austenitized at  $1,500^{\circ}$  F. for one hour  
Quenched to room temperature

| Temp. of draw,<br>° F. | Austen-<br>itizing<br>temp.,<br>° F. | Tensile<br>strength,<br>p.s.i. | Izod<br>impact<br>70° F.<br>ft.-lbs. | Hardness |     |     | Warp-<br>age |
|------------------------|--------------------------------------|--------------------------------|--------------------------------------|----------|-----|-----|--------------|
|                        |                                      |                                |                                      | S        | MR  | C   |              |
| Hot roll.....          | 1,500                                | 205,000                        | 23.7                                 | 636      | 429 | 438 | $\pm .263$   |
| Cold drawn.....        | 1,500                                | 256,500                        | 25.3                                 | 636      | 502 | 470 | $\pm .211$   |
| 640.....               | 1,500                                | 216,000                        | 32.3                                 | 626      | 429 | 402 | $\pm .208$   |
| 1,000.....             | 1,500                                | 204,000                        | 29.7                                 | 619      | 429 | 386 | $\pm .256$   |

Also included among the processes of heat treating after elevated temperature drawing is the process of stress relieving after elevated temperature drawing. This cycle representative of the teachings of this invention will be illustrated using C-1144 steel as before.

The steel after pickling and liming is drawn at elevated temperatures, allowed to cool to room temperature and subsequently reheated to the stress relieving temperature. Tables III and IV will illustrate results obtained using such a cycle with two different percent reductions in area.

Table III

[C-1144 steel drawn to take a 20.3 percent reduction]

| Temp. of<br>draw, ° F. | Stress<br>relief<br>temp., ° F. | Tensile<br>strength,<br>p.s.i. | Yield<br>strength,<br>p.s.i. | Elonga-<br>tion,<br>percent | Red. of<br>area,<br>percent |
|------------------------|---------------------------------|--------------------------------|------------------------------|-----------------------------|-----------------------------|
| 700                    | 1,000                           | 145,000                        | 144,000                      | 9.5                         | 34                          |
| 700                    | 1,000                           | 130,000                        | 110,000                      | 15.0                        | 40                          |

Table IV

[C-1144 steel drawn to take a 35.6 percent reduction]

| Temp. of<br>draw, ° F. | Stress<br>relief<br>temp., ° F. | Tensile<br>strength,<br>p.s.i. | Yield<br>strength,<br>p.s.i. | Elonga-<br>tion,<br>percent | Red. of<br>area,<br>percent |
|------------------------|---------------------------------|--------------------------------|------------------------------|-----------------------------|-----------------------------|
| 700                    | 1,000                           | 156,000                        | 145,000                      | 11.5                        | 29                          |
| 700                    | 1,000                           | 141,000                        | 120,000                      | 11.0                        | 35                          |

It is to be understood that other temperatures than those illustrated in Tables III and IV may be used in the teachings of this invention and although not the same, rolling of the steel may be carried out at the elevated temperature to produce similar results.

It will be apparent from the foregoing examples that steels having new and different properties are secured by

the processing of the steels to take an elevated temperature reduction step followed by heat treating, as by austenitizing and quenching, stress relieving, etc. Steels having reduced stress relationships and improved impact strength are secured while maintaining the strength levels of the steel at a high level.

It will be understood that changes may be made in the details with respect to the methods of heating and cooling the steel, or in the techniques of processing the steel through the various steps embodying the practice of the invention without departing from the spirit of this invention, especially as defined in the following claims.

I claim:

1. The metallurgical process for treating a hot rolled steel which strain hardens and hardens by some mode of precipitation when worked at a temperature between 200° F. and the lower critical temperature for the hot rolled steel composition, consisting of the following combination of steps in the order specified of advancing the steel through a die to effect reduction in cross-sectional area while the steel is at a temperature within the range of 450° F. to the lower critical temperature for the steel composition, subjecting the steel to diffusion transfer subsequent to the elevated temperature reduction step followed by cooling to room temperature.

2. A steel product having new and improved physical and mechanical properties produced by the method of claim 1.

3. The metallurgical process for treating a hot rolled steel which strain hardens and hardens by some mode of precipitation when worked at a temperature between 200° F. and the lower critical temperature for the hot rolled steel composition, consisting of the following combination of steps in the order specified of advancing the steel through a die to effect reduction in cross-sectional area while the steel is at a temperature within the range of 450° F. to the lower critical temperature for the steel composition, carburizing the steel and then cooling the steel to room temperature.

4. The metallurgical process for treating a hot rolled steel which strain hardens and hardens by some mode of precipitation when worked at a temperature between 200° F. and the lower critical temperature for the hot rolled steel composition, consisting of the following combination of steps in the order specified of advancing the steel through a die to effect reduction in cross-sectional area while the steel is at a temperature within the range of 450° F. to the lower critical temperature for the steel composition, nitriding the steel and then cooling the steel to room temperature.

5. The metallurgical process for treating a hot rolled steel which strain hardens and hardens by some mode of precipitation when worked at a temperature between 200° F. and the lower critical temperature for the hot rolled steel composition, consisting of the following combination of steps in the order specified of advancing the steel through a die to effect reduction in cross-sectional area while the steel is at a temperature within the range of 450° F. to the lower critical temperature of the steel composition, cyaniding the steel and then cooling the steel to room temperature.

6. The metallurgical process for treating a hot rolled steel which strain hardens and hardens by some mode of precipitation when worked at a temperature between 200° F. and the lower critical temperature for the hot rolled steel composition, consisting of the following combination of steps in the order specified of advancing the steel through a die to effect reduction in cross-sectional area while the steel is at a temperature within the range of 450° F. to the lower critical temperature for the steel composition, chromizing the steel and then cooling the steel to room temperature.

7. The metallurgical process for treating a hot rolled steel which strain hardens and hardens by some mode of precipitation when worked at a temperature between 200° F.

F. and the lower critical temperature for the hot rolled steel composition, consisting of the following combination of steps in order specified of advancing the steel through a die to effect reduction in cross-sectional area while the steel is at a temperature within the range of 450° F. to the lower critical temperature for the steel composition, carbonitriding the steel and then cooling the steel to room temperature.

8. The metallurgical process for treating a steel which strain hardens and hardens by some mode of precipitation when worked at a temperature between 200° F. and the lower critical temperature for the steel composition consisting of the following combination of steps in the order specified of advancing the steel through a draw die to effect a reduction in cross-sectional area while the steel is at a temperature within the range of 450° F. to the lower critical temperature for the steel composition, subjecting the steel to diffusion transfer subsequent to the elevated temperature reduction step, followed by cooling to room temperature.

9. The metallurgical process for treating a steel which strain hardens and hardens by some mode of precipitation when worked at a temperature between 200° F. and the lower critical temperature for the steel composition consisting of the following combination of steps in the order specified of advancing the steel through a draw die to effect reduction in cross-sectional area while the steel is at a temperature within the range of 450° F. to the lower critical temperature for the steel composition, carburizing the steel, and then cooling the steel to room temperature.

10. The metallurgical process for treating a steel which strain hardens and hardens by some mode of precipitation when worked at a temperature between 200° F. and the lower critical temperature for the steel composition consisting of the following combination of steps in the order specified of advancing the steel through a draw die to effect reduction in cross-sectional area while the steel is at a temperature within the range of 450° F. to the lower critical temperature for the steel composition, nitriding the steel, and then cooling the steel to room temperature.

11. The metallurgical process for treating a steel which strain hardens and hardens by some mode of precipitation when worked at a temperature between 200° F. and the lower critical temperature for the steel composition consisting of the following combination of steps in the order

specified of advancing the steel through a draw die to effect reduction in cross-sectional area while the steel is at a temperature within the range of 450° F. to the lower critical temperature for the steel composition, cyaniding the steel, and then cooling the steel to room temperature.

12. The metallurgical process for treating a steel which strain hardens and hardens by some mode of precipitation when worked at a temperature between 200° F. and the lower critical temperature for the steel composition consisting of the following combination of steps in the order specified of advancing the steel through a draw die to effect reduction in cross-sectional area while the steel is at a temperature within the range of 450° F. to the lower critical temperature for the steel composition, chromizing the steel, and then cooling the steel to room temperature.

13. The metallurgical process for treating a steel which strain hardens and hardens by some mode of precipitation when worked at a temperature between 200° F. and the lower critical temperature for the steel composition consisting of the following combination of steps in the order specified of advancing the steel through a draw die to effect reduction in cross-sectional area while the steel is at a temperature within the range of 450° F. to the lower critical temperature for the steel composition, carbonitriding the steel, and then cooling the steel to room temperature.

#### References Cited in the file of this patent

#### UNITED STATES PATENTS

|    |           |                |                |
|----|-----------|----------------|----------------|
| 30 | 2,183,358 | Six            | Dec. 12, 1939  |
|    | 2,462,851 | Fawcett et al. | Mar. 1, 1949   |
|    | 2,531,731 | Hibbert        | Nov. 28, 1950  |
|    | 2,717,846 | Harvey         | Sept. 13, 1955 |
| 35 | 2,767,837 | Nachtman       | Oct. 23, 1956  |

#### OTHER REFERENCES

Dunn: Iron & Steel Eng., pages 51-57 and 77, July 1946.  
Pomp: The Manufacture and Properties of Steel Wire, 1941, English ed., 1954, pages 92-93.

40 Metals Handbook, pp. 684-685, 1948 edition.  
The Manufacture and Properties of Steel Wire, pp. 58 and 252-256, Pomp, 1954.

The Manufacture and Properties of Steel Wire, Pomp, 45 page 93, 1954.